

Patented June 12, 1923.

1,458,493

# UNITED STATES PATENT OFFICE.

LOUIS MAUERHOFER, OF NEW YORK, N. Y.

## VARNISH COMPOSITION.

No Drawing.

Application filed January 22, 1923. Serial No. 614,294.

To all whom it may concern:

Be it known that I, LOUIS MAUERHOFER, a native of Switzerland, and a resident of the borough of Manhattan, city, county, and

5 State of New York, have invented a new and useful Varnish Composition, of which the following is a specification sufficient to enable those skilled in the art to which the invention appertains to utilize the same.

10 The object of my invention is the production of a varnish capable of general use, but designed more particularly as a polish and protection for metallic surfaces, in that it prevents oxidization and corrosion.

15 To this end, my invention consists of a composition of matter containing the following ingredients in approximately or substantially the relative proportions specified in the formula herein contained, namely,

20 coal tar, benzine and nitric acid combined as a unitary commercial product, it being understood that the quantity of component

parts may be varied somewhat according to special requirements without departing from the spirit and intent of my invention 25 in this respect.

With this understanding, I will state that the following formula is that preferred for general use, to wit:—

About seventy-five (75%) per cent of coal 30 tar, eighteen (18%) per cent of benzine, and seven (7%) per cent of nitric acid.

What I claim as my invention and desire to secure by Letters Patent is,

As an article of manufacture, a varnish 35 of the character designated, composed of coal tar, benzine and nitric acid in substantially the relative proportions herein specified.

LOUIS MAUERHOFER.

Witnesses:

MARIE GABRIELLE MOREL RICKEMAN,  
GEO. WM. MIATT.